

## UNITED STATES PATENT OFFICE

2,004,483

## TREATMENT OF ALLOYS

Edmund F. Bainbridge, Albany, N. Y.

No Drawing. Application January 7, 1930,  
Serial No. 419,211

1 Claim. (Cl. 148—16)

My invention relates to the heat treatment of alloys and particularly steel or iron alloys containing elements which are adapted to or do form carbides harder than the alloy itself. It also relates to a method of heat treating ferrous alloys whereby scale formation is greatly reduced.

In order to roll, forge or otherwise work certain steels or irons it is necessary to heat treat the same at temperatures ranging from above 10 1600 degrees F. to 2500 degrees F. According to the present methods of procedure it is usual to heat these alloys in suitable furnaces but without observing any particular precautions in respect to the character of the atmosphere in which the 15 heating is done. As a result of such treatment there is formed upon the surface of the billets, ingots or bars a considerable quantity of very hard scale which, when analyzed, is found high in carbon as compared with the materials treated. For 20 example, the analysis of the scale so formed upon a billet containing chromium with only 0.07% carbon has indicated a carbon content as high as 0.23%. This scale, or at least some of the constituents thereof, cannot be removed by ordinary 25 pickling acids, and unless removed by physical means, will persist through the subsequent manipulations of the billet and be found in the very finest wire or the smallest rods when the billets have been finally worked to those forms.

Without limiting the scope of my invention in any way by the expression of a definite theory as to the formation of such scale, I believe, that the undesirable demarcations appearing in the final products are due to the presence of hard 30 carbides in the scale. Chrome carbide, for example, which is extremely hard and capable of cutting a sapphire, is probably formed by the reaction of chrome-oxide in the scale with carbon particles in an atmosphere containing little or no uncombined oxygen. Due to its extreme hardness and the fact that it is embedded in or held to the surface of the alloy metal by the other constituents of the scale, it scores the relatively soft

iron or steel during the drawing, forging or other working operations, thus producing the pits and scratches invariably found in the surface of the finished product.

I find that this condition may be overcome by 5 the rather simple expedient of heating the iron or steel to the required temperatures in an atmosphere which is either neutral or contains uncombined oxygen, or which may be generally defined as a non-reducing atmosphere. It is also 10 advantageous to keep the atmosphere surrounding the iron or steel free from solid carbon particles, and to maintain an excess of oxygen there- 15 in to prevent the incipient formation of carbides by the reaction of carbon oxides or hydrocarbon combinations, with the carbide forming element or elements when heated under oxidizing conditions.

In addition to preventing the formation of hard carbides on the surface of the material, thereby 20 eliminating surface pits and scores in the finished product, it will be found that the quantity of scale formed on the material during the heat treatment above described is very much less than that formed on material after treatment by the 25 usual methods.

What I claim is—

The method of preventing pits and scores in a finished product made from an alloy containing 30 chromium which comprises heating the alloy to a hot-working temperature between 1600° F. and 2500° F. adapting it to be rolled or forged, maintaining about the alloy throughout the heating thereof within said temperature ranges an atmosphere substantially free of carbon particles 35 by supplying oxygen to said atmosphere in quantities sufficient to combine with any carbon particles in said atmosphere but not enough to decarburize the alloy substantially, removing the alloy from the heat when the desired working 40 temperature has been reached, and thereafter hot-working it.

EDMUND F. BAINBRIDGE.